

B. BOYKIN, JR.  
METHOD OF CASTING CHILLED VALVE SEATS.  
APPLICATION FILED DEC. 16, 1918.

1,296,751.

Patented Mar. 11, 1919.

*Fig. 1.*



*Fig. 2.*



*Fig. 3.*



*Fig. 4.*



*Inventor*  
*Burwell Boykin, Jr.*

*Witness*

*By* *C. A. Snodgrass*  
*Attorneys*

# UNITED STATES PATENT OFFICE.

BURWELL BOYKIN, JR., OF BEAUMONT, TEXAS.

## METHOD OF CASTING CHILLED VALVE-SEATS.

1,296,751.

Specification of Letters Patent. Patented Mar. 11, 1919.

Application filed December 16, 1918. Serial No. 267,014.

To all whom it may concern:

Be it known that I, BURWELL BOYKIN, Jr., a citizen of the United States, residing at Beaumont, in the county of Jefferson and 5 State of Texas, have invented a new and useful Method of Casting Chilled Valve-Seats. of which the following is a specification.

This invention relates to valve seats and to a method of casting the same, one of its 10 objects being to provide a one-piece seat the active face of which is hardened by chilling during the casting operation, thereby to increase its wearing qualities.

A further object is to provide means 15 whereby, when the molten metal is poured into the mold, a portion thereof will be chilled, the chilling means being retained in the mold for use in successive casting operations.

With the foregoing and other objects in view which will appear as the description proceeds, the invention consists of certain 20 novel features and in the novel steps in the method of making the seats, as will be hereinafter more fully described and claimed, it being understood that various changes may 25 be made in the apparatus used and in the method pursued, without departing from the spirit or sacrificing any of the advantages of the invention as set forth in the 30 appended claim.

In the accompanying drawings the preferred form of the invention and the apparatus used in carrying out the method 35 have been shown.

In said drawings

Figure 1 is a plan view of the drag of the mold with the chills therein.

Fig. 2 is a bottom plan view of the cope.

40 Fig. 3 is a vertical section through the assembled mold ready to receive the molten metal.

Fig. 4 is a section through a valve seat such as produced by the mold.

Referring to the figures by characters of reference, 1 designates the drag filled with sand, as ordinarily. Embedded in the sand 2, at desired points, are chills 3 which can be circular plates, as shown, the upper faces of the chills, if desired, being raised slightly 45 above the surface of the sand 2. Patterns, not shown, are adapted to be placed on the chills, after which sand is placed in the cope 4 and thoroughly packed. The cope is lifted, the patterns removed, and the cope replaced 50 on the drag. Molten metal is then poured into the gate 5 and will be distributed to the various runways 6 and the blanks 7, completely filling them. The hot metal comes 55 into contact with the chills before the blanks are filled and when the operation is completed, the cope is removed, the cast articles 60 lifted from the mold, and the foregoing operation repeated. It is to be understood that the chills are not removed from the mold. 65 A valve seat, such as produced in the manner described is formed with a hardened wear portion, as shown at 8 in Fig. 4 and will be superior to seats made in the usual manner.

70 What is claimed is:—

The herein-described method of producing valve seats which consists in embedding a chill plate in the sand of a drag with its face exposed, placing a pattern on the chill plate, 75 packing sand in a cope and about the pattern, removing the pattern to form a blank closed at the bottom by the chill plate, and supplying molten metal to the blank.

In testimony that I claim the foregoing 80 as my own, I have hereto affixed my signature in the presence of two witnesses.

BURWELL BOYKIN, JR.

Witnesses:

THOS. F. NEESON,  
E. L. BOYKIN.